

March 29, 1949.

H. S. AVERY

2,465,780

Filed Aug. 23, 1946

## HEAT RESISTANT ALLOYS

2 Sheets-Sheet 1



March 29, 1949.

H. S. AVERY

2,465,780

HEAT RESISTANT ALLOYS

Filed Aug. 23, 1946

2 Sheets-Sheet 2

FIG.2.



INVENTOR.  
HOWARD S. AVERY  
BY

*J. M. Nolan*  
ATTORNEY

## UNITED STATES PATENT OFFICE

2,465,780

## HEAT-RESISTANT ALLOYS

Howard S. Avery, Mahwah, N. J., assignor to  
American Brake Shoe Company, New York,  
N. Y., a corporation of Delaware

Application August 23, 1946, Serial No. 692,589

5 Claims. (Cl. 75—128)

1

This invention relates to high strength heat resisting alloys, and more particularly to iron base alloys including chromium, nickel, nitrogen, columbium and carbon.

An object of this invention is to provide a heat resisting alloy characterized by high load carrying ability at elevated temperatures particularly in the range from 1200° F. to 1800° F.

Another object of this invention is to provide an alloy which is resistant to hot gas corrosion and which has a low rate of deformation under stress at high temperatures and a good life expectancy at high stresses.

Another object of this invention is to obtain alloys having high strength and oxidation resistance at elevated temperatures with a minimum of such strategic elements as cobalt, tungsten, molybdenum, columbium, chromium and nickel. Of these, cobalt, tungsten and columbium are quite expensive, and, if required in large percentages, render the resulting alloy too costly for many industrial applications.

Iron base alloys containing substantial amounts of chromium and nickel have been generally found to be satisfactory for heat resisting service, the grade known as 26:12 (containing about 26% chromium and 12% nickel, and known as Alloy Casting Institute Type "HH") in particular providing perhaps the most economical combination of hot gas corrosion resistance and elevated temperature strength. This grade, in the form of castings, is usually produced within the range described by ASTM Specification B190-44T as follows:

| C percent | Mn percent | Si percent | Ni percent | Cr percent | N percent | P percent | S percent | Balance |
|-----------|------------|------------|------------|------------|-----------|-----------|-----------|---------|
| 0.20      | 2.5 max.   | 1.75 max.  | 10         | 23         | 0.20 max. | 0.05 max. | 0.05 max. | Iron    |
| 0.45      |            |            | 14         | 28         |           |           |           |         |

The corresponding wrought alloys customarily contain lower chromium and carbon contents.

If the working stresses of such cast or wrought alloys are low, they may be expected to give long satisfactory service. If service stresses are high, however, they may soon become unserviceable through excessive deformation (creep) or through fracture. Their strength is subject to control over a wide range (represented by limiting creep stress (L. C. S.) values from 300 to 3,000 P. S. I. at 1800° F.) by adjustment of the components of the alloy. The chief factor for obtaining an L. C. S. of above 2200 P. S. I. at 1800° F. is carbon content. Below this level, the proper balance of all alloying elements is helpful, the balance being judged by the freedom from ferrite development in certain temperature ranges. ("Engineering Properties of Heat Resistant Al-

loys," by Howard S. Avery, Earnshaw Cook and J. A. Fellows, A. I. M. E. Technical Publication No. 1480, Metals Technology, August 1942, and Trans. A. I. M. E., vol. 150 (1942), pp. 373-400.)

For high service stresses, it is possible to provide greater than usual strength by manufacturing within the carbon range from 0.40% to 0.50%. However, the brittle nature of these alloys has led to their virtual abandonment in commercial practice. The brittleness of these alloys at room temperature has been held responsible for service failures, but a more careful analysis and appropriate testing have indicated that their chief disadvantage is a short life expectancy at stresses imposed to take advantage of their low deformation rates at high temperature. Stated differently, their creep strength is high, but rupture strength and life expectancy are relatively poor.

20 A survey of the 26% Cr : 12% Ni alloys described in the prior art indicates that they are limited to stresses below 4000 P. S. I. at 1800° F. or fracture in less than 1000 hours may be expected, and similarly limited to below 13,000 P. S. I. at 1400° F. If minimum deformation rates of less than 1% per 10,000 hours are required the alloys are restricted to below 3000 P. S. I. at 1800° F. and 10,000 P. S. I. at 1400° F.

25 In accordance with this invention, alloys are provided that have minimum creep properties that equal or exceed the maximum creep properties of the prior art as described above. The alloys of this invention have compositions including .4% to .8% carbon and preferably from

.45% to .55% carbon, not greater than 1.5% manganese and preferably from .5% to 1.5% manganese, not greater than 1.5% silicon and preferably .2% to 1.5% silicon, 13% to 22% nickel and preferably 13% to 16% nickel, 25% to 31% chromium and preferably 25% to 28% chromium, .04% to .20% nitrogen and preferably .08% to .18% nitrogen, .85% to 2.1% columbium and preferably 1.0% to 1.5% columbium and the remainder chiefly iron. It is essential that this alloy be austenitic; i. e., substantially free from ferrite. If this condition does not obtain, it is expected to be too weak for the purpose intended. To insure production in the austenitic range, the alloys of this invention should have an alloy index not greater than 3.2 and preferably below 2.5 when the percentage of each of the constit-

uents of the alloy is substituted in the following formula:

$$\text{Alloy index} = (.46 \times \% \text{ Cr} + .7 \times \% \text{ Si} + 2 \times \% \text{ Mn} + 1.3 \times \% \text{ Cb}) - (.56 \times \% \text{ Ni} + 6.2 \times \% \text{ C} + 10.0 \times \% \text{ N})$$

The alloys of this invention are characterized by being substantially austenitic and have a permeability of less than 1.05. They have an L. C. S. (limiting creep stress) at 1400° F. of at least 10,000 pounds per square inch; an L. C. S. at 1800° F. of at least 3,000 pounds per square inch; an L. R. S. (limiting rupture stress) for 1,000 hours at 1400° F. of at least 13,000 pounds per square inch; and an L. R. S. for 1,000 hours at 1800° F. of at least 4,000 pounds per square inch.

The alloys of this invention may be produced by conventional means in electric arc or induction furnaces if good steel making practice is followed. The heats reported hereinafter were made in basic lined furnaces, by charging low-carbon steel, ferrosilicon, nickel shot, low-carbon ferrochromium, nitrogen - bearing ferrochromium, high-carbon ferrochromium, ferromanganese, and ferrocolumbium in amounts calculated to yield the desired final analysis. The ferromanganese and ferrosilicon may be reserved until after the melt down. Addition of the silicon as 50% ferrosilicon about two minutes before tapping is generally sufficient for deoxidation. While furnace practice is not critical, it is essential that the skill of the melter be exercised to produce clean, gas free metal.

This material is intended primarily for casting. If hot working is desired, it must be carried out at a very high temperature because of the great hot strength of the alloys.

The data on elevated temperature properties of the specific alloys hereinafter described were obtained on as cast specimens, and the alloys might be used in this condition. If undesirable internal stresses are present after casting, they may be partially relieved and reduced to tolerable levels by heating at 1800° F. for six hours, followed by slow cooling. This treatment is recommended if critical machining is to be done.

If service temperatures below 1800° F. are contemplated and dimensional stability is important, an aging treatment for twenty-four hours at the intended service temperature may be advisable. This causes some carbide precipitation and consequent contraction, but experimental evidence indicates that after twenty-four hours dimensions are relatively constant.

Several methods have heretofore been proposed for producing a 26% Cr : 12% Ni alloy involving the utilization of a formula for the determination of the alloy balance. One such method involves the amount of chromium, car-

bon and nickel in the alloy in accordance with the following formula:

$$\frac{\text{Cr} - 16\text{C}}{\text{Ni}} = \text{ratio factor}$$

The ratio factor according to the authors of this method should be below 1.7, if a substantially austenitic alloy is to be obtained. This formula fails to include the effect of other elements, particularly nitrogen, and consequently is valid for only one nitrogen level. It is also not correlated with the limiting creep strength over a range of the latter. It is useful, however, for determining if the limiting creep stress at 1800° F. is probably above or below the 2000 pounds per square inch level. Moreover, the authors of this formula point out that carbon contents above .45% are unsatisfactory. While this ratio factor method of composition control may be used to produce alloys of about 2000 pounds per square inch at 1800° F. or somewhat above, there is no evidence to indicate that it makes consistently possible attainments of L. C. S. values above 3000 pounds per square inch, which is the approximate maximum that has been attained in the prior art by the use of relatively high carbon contents.

It has been known for some time that carbon increases the strength of 26% Cr : 12% Ni alloys. This effect is due partially to its austenite stabilizing influence, but it also has an additional strengthening effect that persists even in the substantially austenitic compositions. Thus, increased carbon may confer increased strength in alloys, the permeability of which is 1.00 and which contain no ferrite. Industrial exploitation has usually been confined to the range from 0.25% to 0.40% carbon for general purposes, with occasional use of the range from 0.4% to 0.5% carbon for high strength. The latter compositions are applied cautiously as their high resistance to deformation is associated with relatively poor life expectancy, which prevents full exploitation of their strength. Alloys containing above 0.50% carbon and the customary ranges of other alloying elements manifest poor elevated temperature ductility, short life expectancy, and decreasing creep strength. Consequently, such alloys have been considered undesirable and are seldom produced commercially. Some early attempts to utilize such materials led to disastrous failures because such alloys did not deform in service but failed by sudden brittle fracture. Current metallurgical literature and past experience with the addition of carbon beyond about 0.40% have discouraged the formulation of alloys containing carbon contents above this value. The effect of carbon on 26% Cr : 12% Ni alloys is indicated by experimental evidence in Table 1.

TABLE 1  
Effects of carbon on 26.3% Cr : 11.3% Ni  
heat resistant alloys

| Alloy | C, percent | Mn, percent | Si, percent | Ni, percent | Cr, percent | N, percent | L. C. S.<br>1800° F.<br>0.0001%<br>per Hr.<br>(1% per<br>10,000 Hrs.)<br>p. s. i. | Room Temperature Properties After Aging for 24 hrs. at 1400° F. — Furnace Cooling |                                               | Elevated Temperature Ductility at 1400° F.<br>20,000 p. s. i.<br>Elongation in percent for 2 inch gauge length |
|-------|------------|-------------|-------------|-------------|-------------|------------|-----------------------------------------------------------------------------------|-----------------------------------------------------------------------------------|-----------------------------------------------|----------------------------------------------------------------------------------------------------------------|
|       |            |             |             |             |             |            |                                                                                   | Tensile Strength, p. s. i.                                                        | Elongation in percent for 2 inch gauge length |                                                                                                                |
| HH19F | 0.19       | .41         | .43         | 11.4        | 26.5        | .08        | 600                                                                               | 83,000                                                                            | 30.0                                          | 26.5                                                                                                           |
| HH31F | 0.31       | .42         | .42         | 11.4        | 26.5        | .07        | 1150                                                                              | 86,000                                                                            | 25.0                                          | 20.0                                                                                                           |
| HH42  | 0.42       | .45         | .45         | 11.3        | 26.1        | .06        | 2200                                                                              | 89,000                                                                            | 12.5                                          | 9.5                                                                                                            |
| HH62A | 0.52       | .53         | .47         | 11.4        | 26.4        | .07        | 2650                                                                              | 95,750                                                                            | 4.0                                           | 2.5                                                                                                            |
| HH61A | 0.61       | .51         | .48         | 11.4        | 26.3        | .07        | 2500                                                                              | 93,900                                                                            | 2.8                                           | 1.5                                                                                                            |

## Creep characteristics at 1800° F.

| Alloy | C, per cent | Load, p. s. i. | Duration, Hours | Minimum Rate per cent per hour | Residual Properties, Room Temp. |                     |                     |
|-------|-------------|----------------|-----------------|--------------------------------|---------------------------------|---------------------|---------------------|
|       |             |                |                 |                                | Tensile Strength, p. s. i.      | Elongation per cent | Permeability (H=24) |
| HH19F | 0.19        | 500            | 1,995           | 0.000040                       | 81,500                          | 27.0                | 2.83                |
| HH31F | 0.31        | 1,000          | 1,342           | 0.000043                       | 81,500                          | 15.0                | 1.81                |
| HH42  | 0.42        | 2,000          | 1,244           | 0.000047                       | 73,500                          | 6.0                 | 1.20                |
| HH52A | 0.52        | 3,000          | 950             | 0.00016                        | Broke in Creep Test             |                     | 1.00                |
| HH61A | 0.61        | 3,000          | 783             | 0.00026                        | Broke in Creep Test             |                     | 1.00                |

While nitrogen, like carbon, strengthens the 26% Cr : 12% Ni alloys, large amounts of it tend to promote formation of a lamellar constituent which may be associated with high short-time strength but relatively low creep strength.

It has been proposed that columbium and silicon be added in combination to promote formation of a sigma phase which may produce precipitation hardening after suitable heat treatments. This condition is usually associated with brittleness at atmospheric temperatures, and, because the sigma phase tends to transform to ferrite at high temperatures, this mechanism is not considered valuable for producing alloys having high strength at elevated temperatures. The HH31FS alloy listed in Table 2, infra, is a composition of this nature and demonstrates the relatively low strength of this combination.

Columbium has been proposed as an addition agent to neutralize or minimize the tendency of carbon to lower the ductility of the alloy as cast and after exposure to elevated temperatures, about 0.5% to 1% columbium being employed to produce room temperature ductility characteristics similar to those of an alloy with perhaps

15 0.08% to 0.16% lower carbon. These recommendations are coupled with the restriction of carbon plus half of the nitrogen to the preferred range from .26% to .38% and a maximum of 0.45%. The authors of this proposal, however, 20 note significantly that this use has "little or no influence on the strength properties" of the base alloy.

This invention differs from the prior art in requiring the simultaneous combination of three 25 factors in the "HH" type of alloys:

1. An alloy having a carbon content from 0.4% to 0.80%,
2. A balanced substantially austenitic alloy, and
3. An alloy having a columbium content of between 0.85% and 2.1%.

Any two of these factors are not sufficient to produce consistently the high strength and life expectancy that represent the characteristics desired in the alloys of this invention.

Typical examples of alloys of this invention, including their chemical composition and mechanical properties, are given in Tables 2 and 3, which also indicate comparable properties of alloys outside the scope of this invention.

TABLE 2  
Stress-rupture life and secondary creep rate comparison of various 26% Cr : 12 Ni type heat resistant alloys

| Alloy Index | Chemical Analysis |              |              |              |              |             |              | Alloy Index | Mu <sup>1</sup><br>H=24 | 1800° F.—Stress-Rupture—8000 p. s. i. |                         |                           |
|-------------|-------------------|--------------|--------------|--------------|--------------|-------------|--------------|-------------|-------------------------|---------------------------------------|-------------------------|---------------------------|
|             | C, per cent       | Mn, per cent | Si, per cent | Ni, per cent | Cr, per cent | N, per cent | Cb, per cent |             |                         | Fracture Time, Hours                  | Creep Rate per cent Hr. | Elongation per cent in 2" |
| HH32A       | .32               | .48          | .46          | 11.5         | 25.9         | .16         |              | 2.3         | 1.00                    | 1.7                                   | 5.7                     | 22                        |
| HH31FS      | .31               | 1.04         | 3.19         | 11.3         | 26.2         | .04         | 2.09         | 8.6         | 9.10                    | 0.7                                   | 40±                     | 83                        |
| HH31Cb      | .31               | .53          | .66          | 10.7         | 27.1         | .16         | .95          | 4.8         | 2.11                    | 2.6                                   | 3.2                     | 22                        |
| HH40F       | .40               | 1.50         | 1.35         | 13.0         | 26.7         | .10         | 1.94         | 5.3         | 1.78                    | 2.0                                   | 7.5                     | 26                        |
| HH38A       | .38               | .51          | .51          | 12.2         | 25.5         | .20         |              | 1.0         | (1.00)                  | 5.1                                   | 1.7                     | 16                        |
| HH32        | .32               | .54          | 1.18         | 12.8         | 26.7         | .16         |              | 2.5         |                         | 3.2                                   | 3.8                     | 22                        |
| HH42        | .42               | .45          | .45          | 11.3         | 26.1         | .06         |              | 2.9         | 1.02                    | 1.6                                   | 5.3                     | 21                        |
| HH45A       | .45               | .54          | .60          | 12.8         | 26.9         | .08         |              | 2.1         | 1.00                    | 4.8                                   | 0.9                     | 6                         |
| HH32A       | .52               | .53          | .47          | 11.4         | 26.4         | .07         |              | 2.3         | 1.00                    | 9.6                                   | 0.12                    | 3                         |
| HH61A       | .61               | .51          | .48          | 11.4         | 26.3         | .07         |              | 1.7         | 1.00                    | 2.4                                   | 0.12                    | 4                         |
| HH21Cb      | .21               | .60          | .57          | 13.8         | 28.5         | .16         | 1.01         | 4.3         |                         | 1.2                                   | 11.0                    | 23                        |
| HH31Cb      | .31               | .48          | .52          | 14.3         | 26.7         | .12         | 1.06         | 3.0         | 1.00                    | 4.4                                   | 2.9                     | 27                        |
| HH37Cb      | .37               | .51          | .63          | 14.2         | 26.7         | .11         | 1.12         | 2.9         | 1.00                    | 11                                    | 1.1                     | 30                        |
| HH38Cb      | .38               | .58          | .58          | 14.2         | 26.4         | .20         | 1.10         | 1.8         |                         | 17                                    | 0.30                    | 21                        |
| HH41Cb      | .41               | .54          | .56          | 14.2         | 26.7         | .12         | 1.08         | 2.5         | 1.00                    | 13                                    | 0.74                    | 20                        |
| HH47N       | .54               | .98          | 1.29         | 14.3         | 26.7         | .15         | 1.34         | 2.3         | 1.00                    | 14                                    | 0.45                    | 21                        |
| HH48N       | .48               | .84          | .71          | 14.5         | 26.2         | .15         | 1.38         | 1.9         | 1.00                    | 23                                    | 0.16                    | 13                        |
| HH53N       | .56               | .83          | .74          | 14.2         | 26.4         | .17         | 0.73         | 0.7         | 1.00                    | 26                                    | 0.17                    | 16                        |
| HH63N       | .63               | 1.10         | .95          | 13.5         | 27.2         | .16         | 1.05         | 1.7         | 1.00                    | 23                                    | 0.30                    | 24                        |
| HH48Cb      | .48               | .50          | .58          | 14.1         | 26.6         | .12         | .99          | 2.0         |                         | 22                                    | 0.34                    | 22                        |
| HH55Cb      | .55               | .53          | .53          | 14.1         | 26.5         | .12         | 1.05         | 1.5         |                         | 22                                    | 0.20                    | 10                        |
| HH64Cb      | .64               | .48          | .49          | 14.0         | 26.6         | .11         | 1.02         | 1.1         |                         | 29                                    | 0.22                    | 17                        |
| HH65Cb      | .65               | .56          | .47          | 14.0         | 26.5         | .10         | 2.09         | 2.5         |                         | 35                                    | 0.11                    | 11                        |
| HH77Cb      | .77               | .46          | .48          | 13.9         | 26.4         | .13         | 1.09         | 0.2         |                         | 35                                    | 0.13                    | 8                         |

<sup>1</sup> Permeability determined after water quenching from 24 hours at 2000° F.

TABLE 3

*Limiting creep stress and limiting rupture stress comparisons at 1400° F. and 1800° F. for various 26% Cr : 12% Ni type alloys*

| Alloy  | Chemical Analysis |              |              |              |              |             |              | Limiting Creep Stress <sup>1</sup> |           | Limiting Rupture Stress <sup>2</sup> |           |
|--------|-------------------|--------------|--------------|--------------|--------------|-------------|--------------|------------------------------------|-----------|--------------------------------------|-----------|
|        | C, per cent       | Mn, per cent | Si, per cent | Ni, per cent | Cr, per cent | N, per cent | Cb, per cent | 1,400° F.                          | 1,800° F. | 1,400° F.                            | 1,800° F. |
| HH32A  | .32               | .48          | .46          | 11.5         | 25.9         | .16         |              | 5,950                              | 1,750     |                                      |           |
| HH27   | .27               | .51          | 1.18         | 12.0         | 25.0         | .04         |              | 4,400                              | 1,750     | 9,000                                | 2,250     |
| HH45A  | .45               | .54          | .60          | 12.8         | 26.9         | .08         |              | 7,800                              | 3,000     |                                      | 2,750     |
| HH31Cb | .31               | .53          | .66          | 10.7         | 27.1         | .16         | .95          | 3,000                              | 1,000     |                                      |           |
| HH19F  | .19               | .41          | .43          | 11.4         | 26.5         | .08         |              | 2,200                              | 600       |                                      |           |
| HH31F  | .31               | .42          | .42          | 11.4         | 26.5         | .07         |              | 3,400                              | 1,150     |                                      | 1,500     |
| HH42   | .42               | .45          | .45          | 11.3         | 26.1         | .06         |              | 6,300                              | 2,200     |                                      | 2,200     |
| HH52A  | .52               | .53          | .47          | 11.4         | 26.4         | .07         |              | 2,650                              | 13,000    |                                      | 3,800     |
| HH61A  | .61               | .51          | .48          | 11.4         | 26.3         | .07         |              | 2,500                              | 11,000    |                                      | 2,800     |
| HH41Cb | .41               | .64          | .56          | 14.2         | 26.7         | .12         | 1.08         | 10,000                             | 4,500     | 14,500                               | 4,000     |
| HH48Cb | .48               | .50          | .58          | 14.1         | 26.6         | .12         | .99          | 13,000                             |           | 16,000                               | 4,800     |
| HH63Cb | .63               | .48          | .49          | 14.0         | 26.6         | .11         | 1.02         |                                    | 3,750     | 14,500                               | 4,600     |
| HH65Cb | .65               | .56          | .47          | 14.0         | 26.5         | .10         | 2.09         | 13,000                             | 3,800     | 16,000                               | 4,700     |
| HH77Cb | .77               | .46          | .48          | 13.9         | 26.4         | .13         | 1.09         | 11,000                             | 3,800     | 16,500                               | 5,100     |

<sup>1</sup> For a minimum or secondary stage creep rate below 0.0001 per cent per hour; Stress in p. s. i.

<sup>2</sup> For a rupture time or life expectancy of 1,000 hours; stress in p. s. i.

The last ten alloys listed in Table 2 and the last five alloys listed in Table 3 are typical examples of the alloys of this invention, and are produced by the method heretofore described.

In Table 2, the alloy index is calculated in accordance with the formula noted above and is given for each alloy. The permeability of each alloy is expressed by the Greek letter mu ( $\mu$ ). The stress-strain-rupture determinations of these alloys are expressed in terms of fracture time or hours under load before rupture. More particularly, these values indicate the time, in hours, required to fracture the alloy at 1800° F. under a stress of 8000 pounds per square inch. The column captioned Creep rate in per cent per hour is the minimum or secondary stage rate of deformation that is characteristic of creep tests. The column captioned Elongation is the percentage increase in length over a two-inch gauge length during the period under stress before fracture occurred. It is a measure of the elevated temperature ductility of the material. The columns captioned Limiting creep stress, in Table 3, represent the stress required to produce a minimum or secondary stage creep rate not greater than 0.0001% per hour elongation at 1400° F. or 1800° F. respectively. These values are derived from the interpolation or extrapolation of several creep and stress-strain-rupture tests plotted logarithmically as shown in Fig. 1 of the drawing. They correspond to a current engineering definition of limiting creep stress for an elongation rate of 1% in 10,000 hours. The columns captioned limiting rupture stress indicate the stress in pounds per square inch that is expected to produce fracture in 1000 hours and is obtained by interpolation or extrapolation of the fracture times from two or more stress-strain-rupture tests plotted logarithmically as illustrated in Fig. 1. The extension of the fracture time plots permits the estimation of maximum life expectancy at any given stress by reading the stress coordinate that intersects this fracture time line. An example of the characteristics at elevated temperature of a typical alloy of this invention is shown in Fig. 1, representing alloy HH41Cb in Table 2. This alloy is near the low side of the range contemplated by this invention.

Figure 1 is a convenient summary of elevated temperature properties as derived from stress-strain-rupture and creep tests. These two are essentially the same except that creep tests continue for comparatively long times under rela-

tively low loads and usually do not produce fracture of the specimen. The stress-strain-rupture tests are scheduled at higher loads and are intended to produce fracture within reasonable time intervals (e. g. up to six weeks). The creep rates of both of these tests are comparable in significance though different in magnitude.

They apparently are related in such fashion that the data from several plot very close to a straight line on logarithmic paper. The lines in Figure 1 that slope downward to the left connect the creep rate points obtained by testing at the loads of 30,000 pounds per square inch, 20,000 pounds per square inch and 10,000 pounds per square inch at 1400° F., and 8000 pounds per square inch, 6000 pounds per square inch and 5000 pounds per square inch at 1800° F. Plotting in this fashion permits the estimation of creep rate at any stress not too far removed from those of the actual test. The intersection of these lines with that designated 0.0001% per hour creep rate determines the limiting creep stress as previously defined.

The fracture times derived from the same tests described above are similarly plotted to produce the lines sloping downward to the right. They permit estimation of the life before fracture at any stress within the range of those employed and also permit an approximate prediction of behavior under stress for time intervals too long to be practical for actual testing. It should be recognized that there is an element of uncertainty in the extrapolation of the fracture time lines to intervals beyond about 2000 hours. Unfortunately, no better method is available for predicting engineering performance without actually conducting the very long-term tests. It obviously is not practical to extend the time of a creep test

under the stress of 7800 pounds per square inch at 1400° F. to determine if the specimen actually breaks at the end of 100,000 hours, as this test would require twelve years for completion. Thus, these extrapolated values are not to be

considered as completely certain predictions of performance, but they do serve the very useful purpose of permitting the comparison of various alloys on the same basis and under conditions that most nearly approximate the requirements of service.

It may be noted that the values for life and creep rate as recorded for alloy HH41Cb in Table 3 appear on the logarithmic plot as shown in Figure 1. The limiting creep stress and limiting rupture stress values in Table 3 are designated

by arrows on Figure 1. The other values for limiting creep stress and limiting rupture stress that appear in both Tables 2 and 3 were derived from plots similar to these.

The engineering properties of the alloys of this invention having marked strength at elevated temperatures are shown graphically in Figure 2, which is a convenient summary of elevated temperature properties as derived from data exemplified in Figure 1. It permits the selection of recommended design stress, limiting creep stress, or limiting rupture stress values at any temperature between the limits of 1400° F. and 1800° F. On the same charts are plotted the values for yield strength and ultimate tensile strength as obtained from conventional tests at elevated temperature. These values are less useful in design, but are sometimes requested by engineers. If parts of these alloys are subjected to hindered contraction, large thermal stresses may develop. These will rapidly decrease because of creep to values that are characteristic of the temperature involved and which may be derived from the line labeled "Hindered contraction stress" on the diagram. This same line also indicates the approximate residual stress level that will result from stress relief annealing for a short period at any temperature within the range indicated. A further description of the significance of the hindered contraction stress is included in A. I. M. E. technical publication No. 1480, entitled Engineering Properties of Heat Resistant Alloys, by H. S. Avery, E. Cook and J. A. Fellows. It will be noted that this diagram is drawn on semi-logarithmic coordinates, as this permits showing the temperature-stress relationships by means of straight lines over the range from 1400° F. to 1800° F.

The lines on the diagram of Fig. 2, with the exception of those labeled "Yield strength" and "Ultimate tensile strength," represent approximate minimum values of the alloys of this invention, and may be employed for design purposes with reasonable assurance of their validity over a wide composition range, provided the restrictions of this invention are adhered to. The lines for yield strength and tensile strength represent average values and are bordered by a stippled zone to indicate the approximate range in these properties that was encountered during testing.

The room temperature mechanical properties and thermal expansion coefficients of the alloys of this invention are detailed in Tables 4 and 5.

TABLE 4  
Room temperature mechanical properties

| Yield Strength 0.2% Set, P. S. I. | Ultimate Tensile Strength, P. S. I. | Elong., percent 2 | Red. Area, percent | Hardness, BHN |
|-----------------------------------|-------------------------------------|-------------------|--------------------|---------------|
| 38000                             | 60000                               | 9                 | 14                 | 174           |
| 60000                             | 97000                               | 19                | 22                 | 196           |

TABLE 5  
Thermal expansion

| Temp. Range, °F. | Coefficient Microinches Per in per °F. | Total Exp., percent |
|------------------|----------------------------------------|---------------------|
| 50-1, 200        | 9.8                                    | 1.08                |
| 80-1, 400        | 10.0                                   | 1.30                |
| 80-1, 600        | 10.3                                   | 1.54                |
| 80-1, 800        | 10.6                                   | 1.80                |
| 80-2, 000        | 11.3                                   | 2.14                |
| 1, 200-1, 600    | 11.5                                   | 0.46                |

The usual commercial 26% Cr : 12% Ni alloys have good oxidation resistance up to 2000° or 2100° F. The columbium-bearing alloys of this invention have less resistance to hot gas attack, and a maximum service temperature of 1800° F. is suggested. If it is proposed to exploit its high strength above 1800° F., it is desirable to increase the chromium content in proportion and use the upper part of the range provided. Oxidation resistance can be increased by additional silicon also. The use of silicon above 1.5% may be required, however, which tends to impair hot strength.

Unless superior oxidation resistance is especially required, it is recommended that production be confined to the range from 25% to 28% chromium. Chromium below 25% may be satisfactory for strength, but results in decreased protection against hot gas attack.

For alloys of this invention, caution is required in the repair or fabrication of parts by fusion welding. The high hot strength minimizes the plastic deformation that operates to relieve the high thermal stresses developed by the sharp temperature gradients of welding. Weaker materials thus have less tendency to crack. Minor welding repairs may be made with a weaker, more plastic alloy, such as American Iron and Steel Institute type alloy 309Cb, containing about 0.80% columbium and low carbon, but hot strength will be sacrificed for freedom from cracking. If the weld metal is to be critically stressed and must have the strength of the casting, it should be made to the same specification. The avoidance of cracking will then depend on the reduction of thermal gradients by preheating, slow welding and other control factors known to welders.

The alloy index formula in accordance with this invention may lead to the inference that the various elements may be substituted for each other within its quantitative limitations. This is true only for controlling the ferrite-austenite balance within the specified limits. A low carbon alloy, as HH31Cb, in Table 2, may be entirely austenitic but nevertheless exhibit hot strength below the minimum required. Thus increased nickel is not a satisfactory substitute for lowered carbon.

Nitrogen is more nearly equivalent to carbon in its strengthening function. Comparison of alloys HH38A with HH42 and HH45A in Table 2 illustrates this in the absence of columbium. With about 1% columbium, HH38Cb versus HH41Cb and HH48Cb permits a similar comparison and also demonstrates the marked strengthening associated with the columbium addition.

In the production control of this high strength alloy, it is intended that the alloy index formula be employed prior to melting and for molten bath adjustments after preliminary chemical analysis. After production chemical analysis may be used to estimate hot gas corrosion resistance, the 25% Cr minimum being important, to detect borderline heats that may be partially ferritic, and to establish that the desired carbon minimum is attained. For a more precise check of the austenite balance a representative sample is held at 1850° F. for twenty-four hours, water quenched, and a 0.250 inch diameter x 1.00 inch long specimen machined from it, being finished preferably by grinding. This is checked in a permeameter as described in "Precision in Creep Testing," A. I. M. E. Technical Publication No. 1443-C (1942), No. 303, by J. A. Fellows, E. Cook and H. S. Avery,

with a magnetizing force of about 24 oersteds; if the permeability is below 1.05, the alloy balance is considered satisfactory.

Precise control of chemical composition, especially near the extreme limits of the constituents of the alloys of this invention, is a vital factor in producing these alloys satisfactorily. As the introduction of columbium into the chromium-nickel-iron alloys may contribute some difficulties in chemical analysis, the following references are included to permit duplication of the results of this invention.

Metals Handbook, 1939, published by the A. S. M.

Analytical methods for:

Carbon, pages 684-685  
Manganese, pages 686-687  
Silicon, pages 692-693  
Chromium, pages 698-699  
Nickel, pages 700-701  
Columbium, pages 708-709

Scott's Standard Methods of Chemical Analysis, fifth edition, vols. I and II. Published by D. Van Nostrand Company.

Carbon, page 1430  
Silicon, page 1446  
Nickel, pages 1452-1453  
Chromium, pages 1445-1446

Chemical Analysis of Iron and Steel, Lundell, Hoffman & Bright, 1931, published by John Wiley & Sons.

Carbon, page 171  
Manganese, pages 193-194  
Silicon, page 261  
Nickel, pages 280-285  
Chromium, pages 291-292  
Nitrogen, page 426

A. S. T. M. Methods, 1936.

Carbon, pages 9-10  
Manganese, pages 14-15  
Silicon, page 27  
Nickel, pages 31-36  
Chromium, pages 36-38

Determination of Soluble and Insoluble Nitrogen in Ferrochromium Corrosion and Heat Resistant Alloys, by C. M. Johnson, in Iron Age, July, 1935. Reproduced by Precision Scientific Co., Chicago, Illinois, in their Bulletin 151A.

It has been found during years of research on these heat resisting alloys that confusing and misleading results are obtained if the chemical analyses reported are not characterized by accuracy and high precision. With very careful attention to details of procedure and technique it is probable that the essential elements in these alloys can be determined within the following limits: Carbon  $\pm 0.01$ ; manganese  $\pm 0.03$ ; silicon  $\pm 0.04$ ; nickel  $\pm 0.15$ ; chromium  $\pm 0.20$ ; nitrogen  $\pm 0.005$ ; columbium  $\pm 0.03$ . To obtain this precision requires the averaging of duplicate determinations. The effect on the alloy index number is sufficient, if all deviations should be in direction of maximum effect, to produce a range of  $\pm 0.36$ . This range, while not desirable, is not too serious as it is considered to be of approximately the same magnitude as the uncertainties in the alloy index formula. However, if analyses are carelessly run

or if data are contributed from a number of sources, the error may be much more serious. As an example: A group of analyses reported from various sources on a number of samples, there being generally four different reports on each sample, covered a range in deviation from the average of 0.01% to 0.20% carbon; 0.01% to 0.61% manganese; 0.01% to 0.65% silicon; 0.10% to 5.5% nickel; 0.20% to 4.2% chromium; and 10  $\pm 0.02$  nitrogen. If these ranges had been employed in alloy index calculations, the variation would have been plus or minus 1.19 in the A. I. number. Some of the reports were obviously out of line with the others; rejection of these, which 15 was made possible by the availability of several analyses, reduced the alloy index spread to plus or minus 0.54.

A recognition of this problem in precision of analysis was included in a past specification for 20 heat resistant alloys, which permitted a deviation on recheck analysis of  $\pm 0.02$  carbon;  $\pm 0.1$  manganese;  $\pm 0.1$  silicon;  $\pm 0.4$  nickel;  $\pm 0.6$  chromium; and  $\pm 0.02$  nitrogen. This 25 latitude would permit variations of plus or minus 1.02 in alloy index number. The above data have been presented to emphasize the necessity for knowing the real chemical composition of the alloy if proper control is to be exercised in production to obtain the strength values of which 30 the material is capable.

The terms and expressions which I have employed are used as terms of description and not of limitation, and I have no intention, in the use of such terms and expressions, of excluding 35 any equivalents of the features shown and described or portions thereof, but recognize that various modifications are possible within the scope of the invention claimed.

What is claimed is:

40 1. A heat resistant alloy having the composition comprising .4% to .8% carbon, not greater than 1.5% manganese, not greater than 1.5% silicon, 13% to 22% nickel, 25% to 31% chromium, .04% to .20% nitrogen and .85% to 2.1% columbium and the remainder essentially iron, said alloy being characterised in having an alloy index as calculated in accordance with the following formula, of not greater than 3.1:

$$50 \text{Alloy index} = (.46 \times \% \text{ Cr} + .7 \times \% \text{ Si} + .2 \times \% \text{ Mn} + 1.3 \times \% \text{ Cb}) - (.56 \times \% \text{ Ni} + 6.2 \times \% \text{ C} + 10.0 \times \% \text{ N})$$

in which formula each constituent in the alloy is indicated by its percentage of the total alloy.

2. A heat resistant alloy having the composition 55 comprising .45% to .55% carbon, .5% to 1.5% manganese, .2% to 1.5% silicon, 13% to 16% nickel, 25% to 28% chromium, .08% to .18% nitrogen, and 1.0% to 1.5% columbium and the remainder essentially iron, said alloy being characterised in having an alloy index, as calculated 60 in accordance with the following formula, of not greater than 3.1:

$$65 \text{Alloy index} = (.46 \times \% \text{ Cr} + .7 \times \% \text{ Si} + .2 \times \% \text{ Mn} + 1.3 \times \% \text{ Cb}) - (.56 \times \% \text{ Ni} + 6.2 \times \% \text{ C} + 10.0 \times \% \text{ N})$$

in which formula each constituent in the alloy is indicated by its percentage of the total alloy.

3. A heat resistant alloy having the composition 70 of about .48% carbon, about 26.6% chromium, about 14.1% nickel, about .12% nitrogen, about .6% silicon, and about 1.00% columbium and the remainder essentially iron.

4. A heat resistant alloy having the composition 75 about .4% to .8% carbon, about 26.3% chromium, about 14% nickel, about .5% silicon, about .11%

nitrogen, and about 1% columbium and the remainder essentially iron.

5. An iron base heat resisting alloy of the 26% Cr : 12% Ni type including 0.40% to 0.80% carbon, 0.04% to 0.20% nitrogen and .85% to 2.1% columbium, said alloy exhibiting after a heat treatment of twenty-four hours at 1850° F. followed by water quenching a magnetic permeability not greater than 1.05%.

10 HOWARD S. AVERY.

## REFERENCES CITED

The following references are of record in the file of this patent:

## UNITED STATES PATENTS

| Number    | Name                | Date           |
|-----------|---------------------|----------------|
| 2,174,025 | Wise et al. -----   | Sept. 26, 1939 |
| 2,223,659 | Harder et al. ----- | Dec. 3, 1940   |
| 2,256,614 | Franks -----        | Sept. 23, 1941 |